

## UNITED STATES PATENT OFFICE

LUDWIG J. CHRISTMANN, OF JERSEY CITY, AND STUART A. FALCONER, OF ELIZABETH, NEW JERSEY, ASSIGNEES TO AMERICAN CYANAMID COMPANY, OF NEW YORK, N. Y., A CORPORATION OF MAINE

## FROTH FLOTATION

No Drawing.

Application filed January 27, 1930. Serial No. 423,892.

This invention relates to the froth flotation of ores and more particularly to a process which involves the use of promoters of flotation which are novel and useful.

It is among the objects of this invention to provide a method for the separation of various minerals from ores containing the same. More particularly it is among the objects of this invention to recover sulfide minerals and oxidized minerals even in very small amounts from ores. By oxidized minerals, we include compounds of heavy metals, such as lead, zinc, copper, etc., in chemical combination with elements or groups of elements other than sulphur, for instance, in the form of oxides, hydroxides, carbonates and the like.

Our invention contemplates the use as a promoter in a froth flotation operation, of the reaction products of carbon bisulphide and a hydrazine. We generally utilize a substituted hydrazine, either of the aryl or alkyl type.

Although many of the promoters may be successfully used in the flotation of sulfide ores, relatively few are effective in the flotation of oxidized minerals. We have discovered that the above mentioned class of compounds, and particularly the dithiocarbazides, are effective not only for sulfide flotation but also for oxide flotation. Although the free carbazole may be used, we prefer to use salts thereof, such salts being generally of an alkaline nature. We may also use such reagents in combination with other promoters and with frothers and conditioners.

In order to prepare the compounds constituting the subject matter of this invention, we may provide a mixture of 55 parts by weight of phenyl hydrazine hydrochloride with 30 parts by weight of carbon disulfide and 50 parts of water. This mixture is cooled in an ice bath and a solution of 33 parts of potassium hydroxide in 50 parts of water is slowly added with stirring.

After all the potassium hydroxide has been added the mixture is filtered and washed. The filtrate is acidified in an ice bath with hydrochloric acid producing a white precipitate which is filtered and washed. The residue from the reaction mixture is dissolved

in an excess of boiling water, filtered, and the filtrate cooled in an ice bath acidified with hydrochloric acid. The white precipitate formed is filtered, washed and dried. These precipitates may be dissolved in alkali solutions to alkali phenyl dithiocarbazide.

The following is an example illustrative of the practice of our invention on a sample of ore of the Anaconda Copper Company. The ore had the following average head analysis

|           | Per cent |
|-----------|----------|
| Copper    | 5.10     |
| Iron      | 12.9     |
| Insoluble | 62.1     |

A sample was stage crushed to minus 20 mesh. A 1200 gram portion of this minus 20 mesh ore and 600 cc. of water with 4 lbs. of lime per ton were ground in a steel laboratory rod mill for a 10 minute period.

The above grind was transferred to a flotation machine of the sub-aeration type and diluted to 22% solids. Reagents were added to the machine as follows:

0.05 lbs. of phenylthiocarbazole made up as sodium salt per ton  
0.03 lbs. of gns #5 steam distilled pine oil per ton

A concentrate was removed for 3 minutes by skimming. An additional 0.03 lbs. of pine oil per ton was added to middling floated for 8 minutes.

## Results obtained

|             |           |    |
|-------------|-----------|----|
| Heads       | 5.17% Cu  | 85 |
| Concentrate |           |    |
| Grade       | 26.98% Cu |    |
| Recovery    | 87.3 % Cu |    |

## Middling

|                   |       |    |
|-------------------|-------|----|
| Grade             | 18.6% | 90 |
| Recovery          | 5.0%  |    |
| Total Cu recovery |       |    |
|                   | 92.3% |    |

In the flotation of oxide ores these reagents are very effective and the following example illustrates our invention in connection with oxidized lead ore.

1200 g. of minus ten mesh ore, 1200 g. of water 5.0 lbs. of crude mono ammonium phosphate per ton of ore were ground in a steel

laboratory rod mill for 12 minutes. The mesh of the feed was 60% minus 200 mesh. The rod mill charge was transferred to a sub-aeration machine and diluted to 22% solids. The reagents are added to the machine and a mineralized froth collected for 20 minutes.

*Reagents in lbs. per ton of ore*

|    |                                  |       |       |
|----|----------------------------------|-------|-------|
| 10 | Ammonium dibutyl dithiophosphate | 1.25  | 1.25  |
|    | Phenyl dithiocarbazole           | 4.0   |       |
|    | Crude mono-ammonium phosphate    | 5.0   | 5.0   |
|    | Percent lead in heads            | 26.6  | 27.2  |
|    | Percent lead in concentrates     | 38.2  | 47.75 |
|    | Percent lead in tails            | 19.59 | 4.88  |
|    | Percent lead in recovery         | 54.5  | 91.4  |

The class of compounds used by us may be denoted by the following structural formula:



20 in which R is the aryl or alkyl group, such as phenyl, tolyl, naphthyl, methyl and the like, or hydrogen; and Me is an alkaline metal such as calcium, ammonium, sodium and the like, or hydrogen.

25 Although we have described our invention setting forth a few specific examples of the promoters which we have found effective and of ores with which we have worked, our invention is broader than the specific disclosure, in that a large number of compounds may be used in accordance with our invention and a large variety of ores may be successfully floated therewith.

Our invention is, therefore, to be construed broadly except as limited by the claims appended hereto.

What we claim is:

1. A method of recovering minerals from ores which comprises subjecting an ore to a froth flotation operation in the presence of a dithiocarbazole as a promoter.

2. A method of recovering minerals from ores which comprises subjecting an ore to a froth flotation operation in the presence of a substituted dithiocarbazole as a promoter.

3. A method of recovering minerals from ores which comprises subjecting an ore to a froth flotation operation in the presence of an aryl dithiocarbazole as a promoter.

4. A method of recovering minerals from ores which comprises subjecting an ore to a froth flotation operation in the presence of a phenyl dithiocarbazole as a promoter.

5. A method of recovering minerals from ores which comprises subjecting an ore to a froth flotation operation in the presence of an alkaline salt of a dithiocarbazole as a promoter.

6. A method of recovering minerals from ores which comprises subjecting an ore to a froth flotation operation in the presence of an alkaline salt of a substituted dithiocarbazole as a promoter.

7. A method of recovering minerals from ores which comprises subjecting an ore to a

froth flotation operation in the presence of an alkaline salt of an aryl dithiocarbazole as a promoter.

8. A method of recovering minerals from ores which comprises subjecting an ore to a froth flotation operation in the presence of an alkaline salt of a phenyl dithiocarbazole as a promoter.

9. A method of recovering minerals from ores which comprises subjecting an ore to a froth flotation operation in the presence of a promoter having the following structural formula



where R is aryl or alkyl or hydrogen and Me is alkaline radical or hydrogen.

In testimony whereof, we have hereunto subscribed our names this 21st day of January, 1930.

LUDWIG J. CHRISTMANN.  
STUART A. FALCONER.

80

85

90

95

100

100

105

110

115

120

125